

No. 681,091.

Patented Aug. 20, 1901.

C. E. ADAMSON.

WAD FOR CARTRIDGES

(Application filed Apr. 11, 1901.)

(No Model.)

*Fig. 1.*



*Fig. 2.*



WITNESSES,

Thomas L. Ryan  
William A. Thonberg

INVENTOR,

Charles E. Adamson  
by  
John V. Allbrown  
ATTORNEY

# UNITED STATES PATENT OFFICE.

CHARLES ELLSWORTH ADAMSON, OF MUNCIE, INDIANA.

## WAD FOR CARTRIDGES.

SPECIFICATION forming part of Letters Patent No. 681,091, dated August 20, 1901.

Application filed April 11, 1901. Serial No. 55,405. (No model.)

To all whom it may concern:

Be it known that I, CHARLES ELLSWORTH ADAMSON, a citizen of the United States, residing at Muncie, in the county of Delaware and State of Indiana, have invented a new and useful Lubricating Gun-Wad, of which the following is a specification.

This invention relates to a lubricating gun-wad wherein the wad is formed of two or more lubricating materials heated together in compounding, so as to become hard when cold, and which will become semiliquid when subjected to heat.

The primary object of the invention is to provide a lubricating-wad which in its normal condition is sufficiently solid or hard to admit it to be used as an interior or exterior wad, the ingredients and consistency of the wad to be such as to be broken up into fragments by the explosion of the shell and to become melted into a lubricating semiliquid from the heat in the gun-barrel. These and other objects not hereinbefore mentioned are accomplished by the compound described and by the construction illustrated in the accompanying drawings, wherein like letters of reference indicate corresponding parts in both views, and in which—

Figure 1 is a perspective view of one of my wads detached from the cartridge; and Fig. 2 is a section through a cartridge, showing my wad in position in front of the shot to be used as an exterior wad.

I have only shown one position of my wad in the cartridge, as it is obvious that the position can be changed indefinitely.

In the drawings, A designates the brass base, in which the paper shell B is secured in the usual manner. C designates the cap; D, the powder; E, the card wad over the powder; F, the felt wads; G, the shot; H, my improved outer or exterior wad, and I the usual crimp for holding the wad in the cartridge.

In compounding the material for the wad I use as a base powdered graphite, which I mix with hot melted paraffin until it becomes a thick paste, the proportions of each being about one pound of graphite to about six ounces of paraffin, or I find it somewhat improved the compound by using four ounces of

paraffin and two ounces of spermaceti, the latter being more hard and brittle than the paraffin and about the same lubricant, but more expensive. The graphite is mixed in the hot melted paraffin or liquid and then rolled into sheets of the desired thickness to make a gun-wad, then cut or stamped out into little round flat disks like shown in Fig. 1, the diameter of the wads being made to suit the different gauges of guns or shells. The cutting or forming of the disks is done while the material is yet warm to prevent them from breaking up. As soon as the wads become cold they are ready for use or for being packed up in boxes for shipments.

It is well known that a gun-barrel becomes heated by being discharged a number of times in succession, and that in so doing a portion of the residue from the burned powder adheres to the dry barrel and becomes baked thereon. Then after getting in this condition the barrel will begin to "lead," which is a natural result from the friction on the shot while being forced over the dry crusty places in the barrel. It is also well known that when a gun-barrel becomes highly heated that it will lead unless kept moist and lubricated, as herein described.

I have found by experiments that a gun-barrel must be provided with a lubricant that has a sufficient amount of oil to prevent the barrel from becoming dry. The intense heat tends to dry and bake the residue from the powder in the barrel, and by combining a fusible oily lubricant with a powdered non-combustible lubricant the moist lubrication is obtained from one ingredient and the combustion of this moist lubricant prevented by the other ingredient.

By the use of my compound I am able to retain the normal smooth condition of the barrel at all times, as the semiliquid lubrication takes place and is supplied at each discharge of a shell.

I do not confine myself to the exact material or the proportions set forth, as I may find other combinations of a non-combustible and semiliquid or liquid lubrication that will produce the desired effect. Nor do I confine myself to making the entire wad of the com-

27  
pound, as it is obvious that an ordinary wad could be entirely coated with the compound or only have its edges coated.

What I claim is—

- 5 1. A lubricating compound for gun-wads consisting of a fusible and a non-combustible material compounded together so as to become hard in its normal condition.
2. A lubricating-wad for cartridges consist-

ing of a non-combustible and a fusible lubricant compounded so as to become hard in its normal condition.

In testimony whereof I have hereunto set my signature in the presence of two witnesses.

CHARLES ELLSWORTH ADAMSON.

Witnesses:

CHARLES P. GOODWINE,  
SAMUEL CONKLIN.